

Aug. 30, 1949.

J. S. STANIER ET AL

2,480,516

METHOD OF CONTROLLING THE RIMMING OF INGOTS

Filed Aug. 1, 1946

Fig. 1.



Fig. 2.



INVENTOR  
John S. Stanier  
and Ernest B. Plott  
by their attorneys  
Stebbins, Black & Webb

Fig. 3.



Fig. 4.



Fig. 5.



## UNITED STATES PATENT OFFICE

2,480,516

METHOD OF CONTROLLING THE RIMMING  
OF INGOTS

John S. Stanier and Ernest B. Plott, Youngstown,  
Ohio, assignors to The Youngstown Sheet and  
Tube Company, Youngstown, Ohio, a corpora-  
tion of Ohio

Application August 1, 1946, Serial No. 687,570

6 Claims. (Cl. 22—200)

1

This invention relates to the casting of ingots from molten metal and, in particular, to the control of the rimming of molten steel while cooling and freezing to solid form in ingot molds.

Steel as now produced commercially is classified according to its degree of effervescent action when cast into ingot molds as rimming, semi-killed, or killed (The Making, Shaping and Treating of Steel by Camp & Francis, 5th ed., 1940, p. 356). Steel of each classification has well recognized advantages and disadvantages. An ingot of killed steel, for example, has a high degree of uniformity in metallurgical composition but does not have the so-called "skin" characteristic of an ingot of rimming steel. This skin is desirable for the reason that it causes the final product to exhibit fewer surface defects than are present in products made of killed steel. Rimmed steel is also desirable for drawing stock and for its good welding properties. Conversely, a rimmed ingot has a non-uniform composition in the top portion. This requires a substantial portion at the top of the ingot to be cropped and scrapped. The upper one-third of the ingot remaining after cropping, furthermore, is not satisfactory for deep-drawing stock and must be scrapped or used for making other products.

We have invented a method of controlling the rimming action of steel in the ingot mold so as to produce ingots of rimmed steel having the high degree of uniformity throughout the top portion characteristic of killed steel but retaining the skin which minimizes surface defects in the finished product. Our invention permits a reduction in the size of the crop and a corresponding increase in the overall yield. What is more important, it makes possible the use of the upper one-third of the ingot left after cropping, for making deep-drawing stock. In a preferred practice of our invention, we suspend an insert of steel, conveniently a piece of plate, in the top of the ingot mold at a level such that it becomes more or less submerged in the bath of molten steel when poured into the mold to the desired final depth. Steel having full rimming properties is then poured into the mold. The insert is partially fused by the heat of the molten metal and becomes integrally united with the ingot as it freezes. Its presence controls and limits the rimming action so that it is terminated before objectionable non-uniformity in the composition of the top of the ingot has been produced.

A complete understanding of the invention may be gained from the following detailed description and explanation which refer to the accompanying

drawings illustrating the preferred practice diagrammatically. In the drawings,

Figure 1 is a plan view of an ingot mold having one form of insert disposed therein;

Figure 2 is a vertical section through the mold and ingot cast therein;

Figures 3 and 4 are views similar to Figures 1 and 2, respectively, showing a modified form of insert; and

Figures 5 and 6 are also views similar to Figures 1 and 2, respectively, showing a still further modification.

Referring in detail to the drawings, an ingot mold 10 is disposed on a stool 11. An insert 12 is suspended in the upper portion of the mold. The insert has a shackle 13 secured thereto through which is passed a supporting crossbar 14 which extends the width of the mold and rests on the upper edge thereof.

The insert 12, as shown, is a piece of steel plate and has a composition similar to that of the steel to be poured into the mold 10 to form an ingot. The insert should weigh from .2 to .5% of the weight of the ingot, if it is desired to produce strip having the best drawing properties from the ingot. For other products, such as patent leveled sheets or tin plate, where flatness and temper are more important than cleanliness and drawing properties, the weight of the insert should be somewhat greater. In a particular instance, the insert used was a triangle formed from  $\frac{3}{4}$ " plate, measuring 20" along its base with an altitude of about 17".

With the insert in place in the mold, molten steel having full rimming properties is poured into the mold substantially to the level of the top of the insert as indicated at 15, forming an ingot 16. While we prefer to suspend the insert in the mold before pouring the ingot, the insert may alternatively be lowered into the bath of molten steel as soon as the pouring has been completed. The insert does not tend to float in the bath of molten metal since it has a greater density than the latter. The function of the insert is to control and limit the rimming action of the steel in the mold and the size and weight of the insert may be varied to produce the desired effect, the object being to prevent continuation of rimming to the point where it causes objectionable non-uniformity in the upper portion of the ingot. The greater the size of the insert, the greater the suppressing effect on the rimming action. No special surface preparation of the insert is necessary. The presence on the insert of the oxide or scale normally resulting from hot rolling is in no way detrimental to the process since it melts immediately and is

carried to the surface of the bath of molten metal by the rimming action.

By suspending the insert in the mold before pouring the molten steel or placing it in the bath as soon as the pouring is completed, the insert is partially fused and finally becomes integrally united with the ingot as the latter freezes. During cooling, inclusions such as sulphur, phosphorus, oxides and silicates move upwardly and inwardly, eventually striking the converging sides of the insert which deflect them laterally into regions 17 adjacent the top of the ingot. The insert, by reducing the amount of rimming which occurs, cuts down the rimming time.

In a specific example of the practice according to our invention, a heat of steel was poured having the following composition: carbon .07%; manganese .37%; phosphorus .007%; sulphur .022%; and the balance substantially iron. An insert such as that shown at 12 was used, composed of steel plate of about the same composition. When the ingot had cooled sufficiently, the mold was stripped therefrom and the ingot cropped in the usual manner. It was found, however, that our invention increased the overall yield of the ingot by from 2 to 3% because the area of non-uniformity did not extend downwardly as far from the top of the ingot as in the case of ingots poured without the insert. It was thus possible to take a shorter crop from the top of the ingot.

The remainder of the ingot after cropping was then cut into thirds and rolled. The stock produced from the top third of the ingot performed satisfactorily in drawing dies, showing a breakage of only 1.03% in making automobile fenders. This figure was better than that for the stock produced in the lower two-thirds which showed a breakage of 1.8%. This is in contrast with normal rimmed steel in which the breakage of the stock produced from the top third of the ingot is much greater than that encountered in the stock produced from the lower two-thirds.

Other forms of inserts may be used as well as the triangle 12. Figures 3 and 4 show an insert 18 of rectangular shape which has generally the same effect, diverting inclusions to laterally spaced regions 17. Figures 5 and 6 show a further modification in which the inserts are cylindrical members 19 disposed side-by-side, the central member being longer than the side members.

Our invention has the advantage that it makes possible the casting of an ingot having a skin characteristic of rimmed steel but with a uniformity similar to that of an ingot of killed steel. The use of full-rimming steel insures the minimum of surface defects and a maximum of cleanliness and ductility. These characteristics are desirable particularly for stock intended for drawing and forming operations. Rimmed steel is also desirable because of its welding qualities. Our invention combines the advantages of rimmed and semi-killed steel and avoids the disadvantages of killed steel.

A further advantage of the invention is that no special surface preparation of the insert is necessary. The insert, furthermore, may be placed in the mold before pouring or immediately thereafter. No measured wait is necessary with the possibility of varying the effects on the freezing of the ingot.

The increased yield and the possibility of using the top third of the ingot for drawing stock are further advantages which have already been men-

tioned. The ability to use the top third of the ingot for high-grade deep-drawing steel obviously represents a substantial increase in the net yield.

While the invention has been described with particular reference to rimming steel, it may also be used in pouring ingot iron which is cast in molds similar to those used for steel ingots.

Although we have described and illustrated but 10 a preferred practice of the invention with slight modifications, it will be understood that changes in the procedure disclosed may be made without departing from the spirit of the invention or the scope of the appended claims.

15 We claim:

1. In a method of controlling the rimming of an ingot, the steps of pouring molten ferrous rimming metal into an ingot mold and not substantially later than immediately after the conclusion of pouring placing in the upper portion only of the mold and fixedly positioning relatively to the mold an insert of solid ferrous metal which partially fuses into the molten metal and serves to move inclusions upwardly and outwardly and to reduce and limit the normal rimming action.

2. In a method of controlling the rimming of an ingot, the steps of pouring molten ferrous rimming metal into an ingot mold and immediately 20 after the conclusion of pouring placing in the upper portion only of the mold and fixedly positioning relatively to the mold an insert of solid ferrous metal which partially fuses into the molten metal and serves to move inclusions upwardly and outwardly and to reduce and limit the normal rimming action.

3. In a method of controlling the rimming of an ingot, the steps of placing in the upper portion only of an ingot mold and fixedly positioning 30 relatively to the mold an insert of solid ferrous metal which partially fuses into the molten metal and serves to move inclusions upwardly and outwardly and to reduce and limit the normal rimming action.

4. In a method of controlling the rimming of an ingot, the steps of pouring molten ferrous rimming metal into an ingot mold and not substantially 40 later than immediately after the conclusion of pouring placing in the upper portion only of the mold and fixedly positioning relatively to the mold a plate of solid ferrous metal which partially fuses into the molten metal and serves to move inclusions upwardly and outwardly and to reduce and limit the normal rimming action.

5. In a method of controlling the rimming of an ingot, the steps of pouring molten ferrous rimming metal into an ingot mold and not substantially 50 later than immediately after the conclusion of pouring placing in the upper portion only of the mold and fixedly positioning relatively to the mold a triangular plate of solid ferrous metal disposed with its apex downward which partially fuses into the molten metal and serves to move inclusions upwardly and outwardly and to reduce and limit the normal rimming action.

6. In a method of controlling the rimming of an ingot, the steps of pouring molten ferrous rimming metal into an ingot mold and not substantially 60 later than immediately after the conclusion of pouring placing in the upper portion only of the mold and fixedly positioning relatively to the mold a triangular plate of solid ferrous metal disposed with its apex downward which partially fuses into the molten metal and serves to move inclusions upwardly and outwardly and to reduce and limit the normal rimming action.

7. In a method of controlling the rimming of an ingot, the steps of pouring molten ferrous rimming metal into an ingot mold and not substantially 70 later than immediately after the conclusion of pouring placing in the upper portion only of the mold and fixedly positioning relatively to the mold an insert of solid ferrous metal having a weight of from .2% to .5% of the weight

of the ingot which partially fuses into the molten metal and serves to move inclusions upwardly and outwardly and to reduce and limit the normal rimming action.

JOHN S. STANIER. 5  
ERNEST B. PLOTT.

## REFERENCES CITED

The following references are of record in the file of this patent: 10

## UNITED STATES PATENTS

| Number  | Name       | Date          | Number    |
|---------|------------|---------------|-----------|
| 190,055 | Maltby     | Apr. 24, 1877 | 867       |
| 284,004 | Hainsworth | Aug. 28, 1883 | 349,687   |
| 745,117 | Rees       | Nov. 24, 1903 | 15 18,516 |

| Name           | Date           |
|----------------|----------------|
| Hunt           | Apr. 4, 1905   |
| Evans          | Sept. 17, 1907 |
| York           | Nov. 28, 1916  |
| Dornin         | Jan. 10, 1939  |
| Belding        | Feb. 13, 1940  |
| Sternberg      | Apr. 16, 1940  |
| Francis et al. | Aug. 25, 1942  |

## FOREIGN PATENTS

| Country       | Date          |
|---------------|---------------|
| Great Britain | 1914          |
| Germany       | Oct. 7, 1877  |
| Germany       | Mar. 8, 1922  |
| Austria       | Dec. 10, 1904 |